

## [54] SIZED CARBON FIBERS CAPABLE OF USE WITH POLYIMIDE MATRIX

[75] Inventor: Robert Edelman, Staten Island, N.Y.

[73] Assignee: Celanese Corporation, New York, N.Y.

[21] Appl. No.: 276,108

[22] Filed: Jun. 22, 1981

[51] Int. Cl.<sup>3</sup> ..... B32B 5/00; B32B 27/06; D02G 3/00

[52] U.S. Cl. ..... 523/205; 428/367; 428/375; 428/378; 523/215; 524/600; 428/473.5

[58] Field of Search ..... 428/367, 375, 378, 474, 428/408; 528/229, 353; 523/205, 215; 524/600

## [56] References Cited

## U.S. PATENT DOCUMENTS

|           |         |              |       |           |
|-----------|---------|--------------|-------|-----------|
| 3,179,634 | 4/1965  | Edwards      | ..... | 428/379   |
| 3,459,706 | 8/1969  | Schweitzer   | ..... | 528/229 X |
| 3,597,301 | 8/1971  | Blanc et al. | ..... | 528/229 X |
| 3,770,539 | 11/1973 | Bullock      | ..... | 428/367 X |
| 3,837,904 | 9/1974  | Hill         | ..... | 428/367 X |
| 3,914,504 | 10/1975 | Weldy        | ..... |           |
| 3,957,716 | 5/1976  | Weldy        | ..... | 524/87    |
| 4,146,668 | 3/1979  | Dorey et al. | ..... | 428/367 X |

## FOREIGN PATENT DOCUMENTS

89061 4/1972 German Democratic Rep. .

## OTHER PUBLICATIONS

"Low Void Composites Based on NR-150 Polyimide Binders" by Gibbs; Hugh H., 28th Annual Technical Conference, 1973, Reinforced Plastics/Composites Institute, The Society of the Plastic Industry, Inc., Section 2D-pp. 1-3.

"The Development of Quality Control Techniques For

NR-150 Polyimide Adhesive and Binder Materials" by Hugh H. Gibbs et al., pp. 11-17, Sample Journal, Jan., Feb., 1979.

Du Pont, NR-150 Polyimide Precursor Solutions, Bulletin No. 783, revised Mar. 1979, "4,4'-Oxydianiline (ODA)".

Primary Examiner—Lorraine T. Kendall  
Attorney, Agent, or Firm—Herbert P. Price

[57]

## ABSTRACT

Carbon fibers are provided which bear an improved finish coating upon the surface which is capable of withstanding the high temperatures (e.g., above 500° F.) commonly encountered during the formation of composite structures employing a polyimide matrix. The sized carbon fibers prior to the curing to form a rigid polyimide coating are flexible, may be readily handled without significant damage, and are amenable to good impregnation with the matrix resin thereby facilitating the formation of quality composite structures. The finish comprises a mixture of selected precursors for the formation of a rigid polyimide (as described). More specifically, the size composition is formed from at least one aromatic diamine, at least one aromatic dianhydride, and at least one aromatic tetracarboxylic acid diester. A film-forming polyamic acid oligomer readily forms and is present as an intermediate reaction product within the finish coating and the aromatic tetracarboxylic acid diester has been found to beneficially serve primarily as a flexibility preserving diluent during the early stages of the polyimide-forming reaction which takes place within the finish coating. The finish is fully compatible with a polyimide matrix.

26 Claims, No Drawings

## SIZED CARBON FIBERS CAPABLE OF USE WITH POLYIMIDE MATRIX

### BACKGROUND OF THE INVENTION

In the search for high performance materials considerable interest has been focused upon carbon fibers. Industrial high performance materials of the future are projected to make substantial utilization of fiber reinforced composites, and carbon fibers theoretically have among the best properties of any fiber for use as high strength reinforcement. Among these desirable properties are corrosion and high temperature resistance, low density, high tensile strength, and high modulus.

Polymeric materials heretofore commonly have been selected as the matrix material in which the relatively delicate carbon fibers are incorporated to form high performance materials with the carbon fibers serving as a light weight fibrous reinforcement. Epoxy resins most frequently have been selected as the matrix material. Additionally, the use of polyimides as the matrix material has been proposed primarily because of the ability of the polyimides to withstand even higher temperatures during use.

In order to improve the handleability of the carbon fibers without undue fiber damage during the formation of composite articles it has been the common practice to apply a flexible size or finish to the surface of the same. See, for instance, the epoxy size disclosed in U.S. Pat. Nos. 3,914,504 and 3,957,716. The sized carbon fibers bearing the epoxy coating are commonly incorporated in an epoxy matrix resin and a rigid composite article is formed upon curing. Epoxy matrix resins are commonly cured at temperatures below approximately 450° F. If higher temperatures are encountered, the physical properties of the resulting composite article tend to be reduced.

There has remained a need for a highly satisfactory size or finish for use with carbon fibers which is capable of withstanding, without decomposition or loss of the desired size qualities, the more severe temperature conditions encountered when a polyimide serves as the matrix resin. For instance, polyimide resins commonly require an extended curing temperature at 550° to 600° F. At such temperatures epoxy sizes can be expected to undergo some level of degradation which can undesirably influence the physical properties of the resulting composite article.

Polyimide sizes also have been proposed in the prior art, but while being capable of withstanding the temperature involved during the curing of a polyimide matrix resin, have nevertheless been deficient in providing the desired improvement in handleability. Accordingly, the handleability of carbon fibers bearing these sizes generally has been very poor. For instance, if one selects as a size composition a common polyimide precursor solution containing at least one aromatic diamine, and at least one aromatic tetracarboxylic acid, and/or at least one aromatic diacid diester, the various components tend to lack the requisite film-forming characteristics to yield a satisfactory size. For instance, the monomers present tend to be dissolved solids and a brittle non-flexible and non-uniform coating tends to be deposited upon the surface of the carbon fibers which lacks those qualities commonly sought in size. This type of size results in extremely high levels of fuzz because of inadequate

fiber protection and renders the weaving of the same virtually impossible.

It is an object of the present invention to provide sized carbon fibers which may be readily handled without undue fuzz formation or damage to the same.

It is an object of the present invention to provide improved sized carbon fibers which are capable of withstanding high temperatures (e.g., above 500° F.) without deleterious results.

10 It is an object of the present invention to provide improved sized carbon fibers which are particularly suited for use in the formation of composite structures wherein a polyimide serves as the matrix material.

15 It is an object of the present invention to provide improved sized carbon fibers which produce minimal fuzz upon handling.

It is an object of the present invention to provide improved sized carbon fibers which are flexible and capable of readily undergoing impregnation with a

20 matrix material.

It is a further object of the present invention to provide an improved carbon fiber reinforced composite structure comprising a polyimide matrix and a polyimide size coating on the carbon fibers which does not 25 result in any substantial diminution in the overall physical properties of the composite structure.

These and other objects, as well as the scope, nature, and utilization of the claimed invention will be apparent to those skilled in the art from the following detailed 30 description and appended claims.

### SUMMARY OF THE INVENTION

A carbon fiber is provided having a flexible coating on the surface thereof in a concentration of approximately 0.3 to 5.0 percent by weight based upon the weight of the carbon fiber of a sizing composition which comprises a polyamic acid oligomer, and is capable of yielding a rigid polyimide at elevated temperatures which is derived from the reaction of at least one aromatic diamine, at least one aromatic dianhydride, and at least one aromatic tetracarboxylic acid diester in which the carboxylic acid groups and ester groups are ortho disposed, wherein the polyamic acid oligomer is an intermediate in the formation of said rigid polyimide.

40 A composite structure is provided comprising a rigid polyimide matrix having carbon fibers incorporated therein which are coated on the surface thereof with approximately 0.3 to 5.0 percent by weight based upon the weight of the carbon fibers of a sizing composition

45 comprising a rigid polyimide coating which is derived from the reaction of at least one aromatic diamine, at least one aromatic dianhydride, and at least one aromatic tetracarboxylic acid diester in which the carboxylic acid groups and ester groups are ortho disposed, 50 wherein a polyamic acid oligomer is formed as an intermediate during the formation of the rigid polyimide coating and is present within a flexible coating comprising the reactants which facilitates impregnation of the coated carbon fibers with the matrix during the formation of the composite structure.

### DESCRIPTION OF PREFERRED EMBODIMENTS

The carbon fibers which are provided with a protective size coating in accordance with the present invention contain at least 90 percent carbon by weight (e.g., 65 at least 95 percent carbon by weight in preferred embodiments) and such carbon may be either amorphous

or graphitic in nature. Suitable carbon fibers are commercially available and commonly are of a relatively low denier per filament of approximately 0.5 to 2 thereby rendering them susceptible to damage during handling in the absence of a satisfactory size coating, particularly if the fibers also possess a relatively high Young's modulus. Representative carbon fibers are disclosed in commonly assigned U.S. Pat. Nos. 3,775,520; 3,900,556; 3,925,524; and 3,954,950.

The carbon fibers prior to sizing may optionally have their surface characteristics modified so as to improve their ability to bond to a resinous matrix material. Representative surface modification processes are disclosed in U.S. Pat. Nos. 3,657,082; 3,671,411; 3,723,150; 3,723,607; 3,754,957; 3,759,805; 3,859,187; 3,894,884; and in commonly assigned U.S. Ser. No. 222,970, filed Jan. 5, 1981.

The carbon fibers prior to sizing are preferably provided as a multifilamentary fibrous material such as a continuous length of a multifilamentary yarn, tow, 20 strand, tape, etc. However, staple carbon fibers or other fibrous assemblages may be satisfactorily sized through the use of the present invention. For best results the configuration of the carbon fibers is such that the surfaces of the individual fibers are substantially exposed 25 when the size composition is applied.

The size composition which forms a flexible size on the surface of the carbon fibers comprises a film-forming polyamic acid oligomer and is capable of yielding a rigid polyimide at elevated temperatures which is derived from the reaction of (1) at least one aromatic diamine, (2) at least one aromatic dianhydride, (3) and at least one aromatic tetracarboxylic acid diester in which the carboxylic acid groups and ester groups are ortho disposed, wherein the polyamic acid oligomer is an intermediate in the formation of the rigid polyimide. The polyamic acid oligomer alternatively can be termed a polyamide acid oligomer.

Representative aromatic diamines are p-phenylenediamine, m-phenylenediamine, 4,4'-oxydianiline, 4,4'-methylenedianiline, 4,4'-diaminodiphenylsulfone, 4,4'-diaminobenzophenone, 4,4'-diaminobiphenyl, 3,3'-diaminodiphenylsulfone, 3,3'-diaminobenzophenone, and mixtures thereof. Particularly satisfactory results have been obtained when a mixture of approximately 95 percent by weight of p-phenylenediamine and approximately 5 percent by weight of m-phenylenediamine is selected. The aromatic diamine reactant preferably is provided in a concentration of approximately 50 mole percent based upon the total concentration of the three classes of reactants.

Representative aromatic dianhydrides are 3,3',4,4'-benzophenonetetracarboxylic dianhydride, pyromellitic dianhydride, 3,3',4,4'-(hexafluoroisopropylidene)-bis(phthalic anhydride), and mixture thereof. Particularly satisfactory results have been obtained when 3,3',4,4'-benzophenonetetracarboxylic dianhydride is selected. The aromatic dianhydride reactant preferably is provided in a concentration of approximately 30 to 40 mole percent based upon the total concentration of the three classes of reactants, and most preferably in a concentration of approximately 35 mole percent based upon the total concentration of the three classes of reactants. The aromatic dianhydride is capable of undergoing an immediate reaction with the aromatic diamine even at ambient conditions to yield a polyamic acid oligomer. Other polyimide-forming reactants such as aromatic tetracarboxylic acids and aromatic diester

diacids have been found to be substantially incapable of undergoing such reaction with the aromatic diamine to form the desired film-forming polyamic acid oligomer. The formation of the film-forming polyamic acid oligomer continues during the application of the size while the size composition is heated while present on the carbon fibers at moderate temperatures, e.g., at approximately 150° C. for approximately 2 minutes as described hereafter.

The aromatic tetracarboxylic acid diester may be formed by known techniques through the reaction of an aromatic dianhydride with an alcohol having 1 to 6 carbon atoms. Representative alcohols for this reaction are methyl alcohol, ethyl alcohol, n-propyl alcohol, isopropyl alcohol, isobutyl alcohol, tert-butyl alcohol, n-amyl alcohol, hexyl alcohol, etc. The preferred alcohol for use when forming the aromatic tetracarboxylic acid diester is ethyl alcohol.

Representative aromatic tetracarboxylic acid diesters are 3,3'-diethylester of 3,3',4,4'-benzophenonetetracarboxylic acid, 3,3'-diethylester of 3,3',4,4'-(hexafluoroisopropylidene)bis(phthalic acid), 1,5-diethylester of pyromellitic acid, and mixtures thereof. Particularly satisfactory results have been obtained when the 3,3'-diethylester of 3,3',4,4'-benzophenonetetracarboxylic acid is selected. The aromatic tetracarboxylic acid diester preferably is provided in a concentration of approximately 10 to 20 mole percent based upon the total concentration of the three classes of reactants, and most preferably in a concentration of approximately 15 mole percent based upon the total concentration of the three classes of reactants. In the present invention the aromatic tetracarboxylic acid diester undergoes only minimal reaction with the aromatic diamine while the coating on the carbon fibers is serving its function as a flexible size. It is only upon heating at more elevated temperatures that the aromatic tetracarboxylic acid diester enters into the polyimide-forming reaction. While present in the size the aromatic tetracarboxylic acid diester beneficially contributes to the desirable properties exhibited by maintaining size flexibility. It serves the key role in the present invention of controlling the development of the desired polyamic acid oligomer. Since this material serves as a reactive diluent, it does not diminish the ultimate cured properties of a polyimide composite because it will react with the other components to form a polyimide during the composite cure cycle. If the aromatic tetracarboxylic acid diester is omitted from the size composition and molar concentration of the aromatic dianhydride correspondingly is increased, then it has been found that the reaction between these two polyamic acid-forming reactants is too extreme and tends to greatly diminish the desired flexibility of the size composition when present upon the carbon fibers at moderate temperatures. The resulting stiffness of the carbon fiber bundles then prevents adequate wetting of the fibers during resin impregnation.

The flexible size coating preferably is applied to the carbon fibers when dissolved in a polar solvent which is incapable of harming the carbon fibers. Representative solvents for the reactants and resulting polyamic acid are N-methyl pyrrolidone, dimethylformamide, dimethylacetamide, dimethylsulfoxide, etc. Such solvents tend to be relatively high boiling (e.g., have a boiling point above approximately 150° C.). In a preferred embodiment a relatively volatile solvent (e.g., having a boiling point below approximately 70° C.) additionally is also present and is believed to aid in the removal of the polar

solvent following contact of the carbon fibers with the dissolved reactants which are capable of forming the desired size. The preferred polar solvent for the reactants is N-methyl pyrrolidone and the preferred volatile solvent is acetone. Particularly satisfactory results are achieved when approximately 30 percent by weight of the solvent mixture is N-methyl pyrrolidone and approximately 70 percent by weight of the solvent mixture is acetone. The total concentration of the reactants present in the solvent mixture when initially contacted with the carbon fibers preferably is approximately 0.6 to 10 percent by weight based upon the total weight of the solution.

The solution which is capable of forming the flexible size coating may be applied to the carbon fibers by any suitable technique such as dipping, padding, etc. The solution preferably is provided at a temperature of approximately room temperature (e.g. approximately 25° C.) when applied to the carbon fibers. Once the solution is applied, the solvent is substantially volatilized by heating in an appropriate zone which is provided at a more highly elevated temperature. The temperature of such zone will be influenced by the boiling point of the polar solvent selected and preferably does not exceed approximately to 150° to 160° C. Heating times of approximately 2 minutes have been found to be satisfactory. Appropriate equipment and safety precautions must be taken to insure the safety of personnel in the area and to effectively deal with the explosion hazard created by solvent vapors. Every effort is made to remove the solvent to the fullest extent possible; however, a minor amount of N-methyl pyrrolidone will still be present in the size composition following such heating.

Upon volatilization of the solvent the size coating is deposited upon the surface of the carbon fiber in a concentration of approximately 0.3 to 5.0 percent by weight based upon the weight of the carbon fiber, and most preferably in a concentration of 0.5 to 1.3 percent by weight based upon the weight of the carbon fiber.

In a preferred embodiment the flexible coating on the surface of the carbon fiber comprises a polyamic acid oligomer, and is capable of yielding a rigid polyimide at more highly elevated temperatures which is derived from the reaction of approximately 47.5 mole percent of p-phenylenediamine, approximately 2.5 mole percent of m-phenylenediamine, approximately 35 mole percent of 3,3',4,4'-benzophenonetetracarboxylic dianhydride, and approximately 15 mole percent of 3,3'-diethylester of 3,3',4,4'-benzophenonetetracarboxylic acid. The polyamic acid oligomer in this instance is formed primarily upon the reaction of the p-phenylenediamine, the m-phenylenediamine, and the benzophenonetetracarboxylic dianhydride to form an oligomer of the following general formula wherein the corresponding moieties derived from m-phenylenediamine are not shown for simplicity of illustration:



where x is a small number, e.g., approximately 2 to 10, or more.

The carbon fiber bearing the flexible size coating in accordance with the present invention may be handled without undue damage. The fuzz problem which commonly exists when one attempts to process continuous lengths of unsized carbon fibers is significantly reduced. Also bundles of carbon fibers bearing the size coating are amenable to flattening and spreading thereby facilitating ready impregnation of the same by the matrix resin during the formation of a composite structure in accordance with standard technology. Such impregnation is believed to result in composite structures possessing improved mechanical properties. Additionally the size coating is highly compatible with a polyimide matrix resin and is capable of withstanding the elevated temperatures for the curing of a polyimide matrix resin (e.g., 500° to 700° F.). Carbon fiber bundles bearing the size of the present invention can be woven without any substantial damage to the relatively delicate carbon fibers.

At the higher temperatures encountered during the formation of a composite article the flexible size coating is transformed into a solid polyimide through the reaction of all of the reactants. Representative polyimide resins which may be employed as the matrix resin during the formation of a composite structure are bismaleimide resins, which are manufactured by Rhone Poulenc under the designation Kerimid 601, 353, and MVR711, and by Technochemie GmbH under the designation M751, M756, and H795; addition condensation polyimides which are manufactured by Hexcel and Kingmar Labs under the designation LaRC 160, and by U.S. Polymeric under the designation PMR 15; and condensation polyimides by E. I. DuPont de Nemours & Co. under the designation NR-150, NR-150A, NR-150A2, NR-150A2G, NR-150A2S5X, NR-150B, NR-056X, NR-058X, etc. The NR-150 polyimide is discussed in "Low Void Composites Based on NR-150 Polyimide Binders" by Hugh H. Gibbs, published at Section 2-D, Page 1 to 3 of the 28th Annual Technical Conference, 1973, Reinforced Plastics Composites Institute, The Society of the Plastics Industry, Inc.; and in "The Development of Quality Control Techniques for NR-150 Polyimide Adhesive and Binder Materials" by Hugh H. Gibbs and John R. Ness, published at Pages 11 to 17 SAMPE Journal, January February 1979. The NR-058X polyimide has been marketed as a polyimide precursor solution containing a polyamide acid based on 4,4'-oxydianiline.

The sized carbon fibers may be impregnated with the composition which forms the matrix resin (1) by contact with a resin film followed by heat and pressure, (2) by pulling through a bath containing molten matrix-forming components, or (3) by coating with a resin solution containing a low boiling solvent which is subsequently removed by running the coated fibers through a heated oven.

The sized carbon fibers following curing preferably are provided in the polyimide matrix resin in a concentration of approximately 50 to 73 percent by volume and most preferably in a concentration of approximately 60 to 65 percent by volume based upon the total volume of the final composite structure.

The resulting composite articles can be utilized as strong lightweight structural components which are capable of service at elevated temperature (e.g., 500° to 600° F.). For instance, the composite articles may serve in aerospace components, particularly for engine appli-

cations, such as engine cowls, engine nacelle, engine oil tank ducts as well as shuttle orbiter aft body flaps, etc.

The following example is presented as a specific illustration of the claimed invention. It should be understood, however, that the invention is not limited to the specific details set forth in the example.

#### EXAMPLE

The carbon fiber selected for sizing was a yarn of carbonaceous filamentary material derived from an acrylonitrile copolymer consisting of approximately 98 mole percent of acrylonitrile units and 2 mole percent methylacrylate units. The carbonaceous material consisted of approximately 6000 substantially parallel filaments, contained approximately 93 percent carbon by weight, and was commercially available from the Celanese Corporation under the designation of Celion 6000. Representative average filament properties for the carbon fiber were a denier of 0.6, a tensile strength of approximately 470,000 psi, a Young's modulus of approximately 34 million psi, and an elongation of approximately 1.4 percent.

To vessel No. 1 were added, at room temperature with stirring, 173.4 parts by weight of N-methyl pyrrolidone, 11.3 parts by weight of p-phenylenediamine, and 0.6 parts by weight of m-phenylenediamine. The p-phenylenediamine and the m-phenylenediamine dissolved in the N-methyl pyrrolidone solvent. While stirring continued, 27.3 parts by weight of 3,3',4,4'-benzophenonetetracarboxylic dianhydride were slowly added and the temperature was allowed to rise to a maximum of approximately 40° C. Stirring continued until the benzophenonetetracarboxylic dianhydride as well as all other components were completely dissolved.

To vessel No. 2 were added, at room temperature with stirring, 25 parts by weight of N-methyl pyrrolidone and 8.31 parts by weight of 3,3',4,4'-benzophenonetetracarboxylic dianhydride. The temperature was raised to 70° C. and stirring continued. When all of the 3,3',4,4'-benzophenonetetracarboxylic dianhydride had dissolved, 2.4 parts by weight of absolute ethyl alcohol were added to the heated solution. A cover was placed over vessel No. 2 to prevent evaporation of the ethyl alcohol, and the temperature was raised to 80° C. and held at that temperature for 30 minutes. This solution which contained the dissolved 3,3'-diethylester of 3,3',4,4'-benzophenonetetracarboxylic acid as a reaction product was cooled to room temperature.

The solution from vessel No. 2 was added to vessel No. 1 with stirring while the contents of vessel No. 1 were at room temperature. The resulting concentrated mixture contained 20.1 percent by weight solids dissolved therein, and was stored under refrigeration until diluted for application as a size or finish to the carbon fibers.

A portion of the concentrated mixture next was diluted with additional N-methyl pyrrolidone and with acetone to form the size solution which was applied to the carbon fibers. The resulting solvent mixture was composed of 70 percent by weight acetone, and 30 percent by weight N-methyl pyrrolidone and the size components were present therein in a concentration of 0.9 percent by weight based upon the total weight of the solution. More specifically, 100 parts by weight of the concentrated mixture were first mixed with 548 parts by weight of N-methyl pyrrolidone and then 1549 parts by

weight of acetone were next dropwise added while stirring to form the final sizing solution.

The resulting dilute size solution was applied to the carbon fiber within one day of its formation. The solution contained a film-forming polyamic acid oligomer which was formed primarily by the reaction of the p-phenylenediamine and the m-phenylenediamine with the 3,3',4,4'-benzophenonetetracarboxylic dianhydride. The 3,3'-diethylester of 3,3',4,4'-benzophenonetetracarboxylic acid present served primarily as an unreacted diluent which was capable of entering into the polyimide-forming reaction at more highly elevated temperatures. The presence of such reactive diluent served to limit the increase in viscosity resulting from the polyamic acid oligomer formation thereby preserving the desired flexibility of the size coating.

More specifically, the sizing of the continuous length of the carbon fibers was accomplished while being dipped within and being passed in the direction of its length at a rate of 5 meters per minute through a metal trough containing the sizing solution at room temperature.

The solvent next was removed from the surface of the carbon fibers by drying for a residence time of two minutes in a circulating air oven provided at 150° C. A flexible coating was provided on the surface of the carbon fiber in a concentration of 0.6 percent by weight, which imparted highly improved handling characteristics to the carbon fibers while significantly reducing the fuzz level. A very small amount of N-methyl pyrrolidone was present within this resulting size coating but did not significantly reduce the properties of the composite article ultimately produced.

The sized carbon fiber was capable of spreading to well accommodate impregnation with a standard polyimide matrix resin system during the formation of a carbon fiber reinforced composite structure. Upon curing the size coating also yields a rigid polyimide which is highly compatible with the polyimide matrix.

Although the invention has been described with a preferred embodiment, it is to be understood that variations and modifications may be employed without departing from the concept of the invention as defined in the following claims.

I claim:

1. A carbon fiber having a flexible coating on the surface thereof in a concentration of approximately 0.3 to 5.0 percent by weight based upon the weight of the carbon fiber of a sizing composition which comprises a polyamic acid oligomer, and is capable of yielding a rigid polyimide at elevated temperatures which is derived from the reaction of at least one aromatic diamine, at least one aromatic dianhydride, and at least one aromatic tetracarboxylic acid diester in which the carboxylic acid groups and ester groups are ortho disposed, wherein said polyamic acid oligomer is an intermediate in the formation of said rigid polyimide.

2. A carbon fiber having a flexible coating on the surface thereof according to claim 1 wherein said coating is present in a concentration of approximately 0.5 to 1.3 percent by weight based upon the weight of the carbon fiber.

3. A carbon fiber having a flexible coating on the surface thereof according to claim 1 which is capable of forming said rigid polyimide through the reaction of approximately 50 mole percent of said at least one aromatic diamine, approximately 30 to 40 mole percent of said at least one aromatic dianhydride, and approxi-

mately 10 to 20 mole percent of said at least one aromatic tetracarboxylic acid diester wherein the carboxylic acid groups and ester groups are ortho disposed.

4. A carbon fiber having a flexible coating on the surface thereof according to claim 1 wherein acid aromatic diamine is selected from the group consisting of p-phenylenediamine, m-phenylenediamine, 4,4'-oxydianiline, 4,4'-methylenedianiline, 4,4'-diaminodiphenylsulfone, 4,4'-diaminobiphenyl, 3,3'-diaminodiphenylsulfone, 3,3'-diaminobenzophenone, and mixtures of the foregoing.

5. A carbon fiber having a flexible coating on the surface thereof according to claim 1 wherein said aromatic diamine is a mixture of approximately 95 percent by weight p-phenylenediamine and approximately 5 percent by weight of m-phenylenediamine.

6. A carbon fiber having a flexible coating on the surface thereof according to claim 1 wherein said aromatic dianhydride is 3,3',4,4'-benzophenonetetracarboxylic dianhydride, pyromellitic dianhydride, 3,3',4,4'-(hexafluoroisopropylidene)bis(phthalic anhydride), and mixtures of the foregoing.

7. A carbon fiber having a flexible coating on the surface thereof according to claim 1 wherein said aromatic dianhydride is 3,3',4,4'-benzophenonetetracarboxylic dianhydride.

8. A carbon fiber having a coating on the surface thereof according to claim 1 wherein said aromatic tetracarboxylic acid diester is formed by the reaction of an aromatic dianhydride and an alcohol having one to six carbon atoms.

9. A carbon fiber having a flexible coating on the surface thereof according to claim 8 wherein said alcohol is ethanol.

10. A carbon fiber having a coating on the surface thereof according to claim 1 wherein said aromatic tetracarboxylic acid diester is the 3,3'-diethylester of 3,3',4,4'-benzophenonetetracarboxylic acid, the 3,3'-diethylester of 3,3',4,4'-(hexafluoroisopropylidene)bis(phthalic acid), the 1,5-diethylester of pyromellitic acid, and mixtures of the foregoing.

11. A carbon fiber having a coating on the surface thereof according to claim 1 wherein said aromatic tetracarboxylic acid diester is the 3,3'-diethylester of 3,3',4,4'-benzophenonetetracarboxylic acid.

12. A carbon fiber having a flexible coating on the surface thereof in a concentration of approximately 0.3 to 5.0 percent by weight based upon the weight of the carbon fiber of a sizing composition which comprises a polyamic acid oligomer, and is capable of yielding a rigid polyimide at elevated temperatures which is derived from the reaction of approximately 47.5 mole percent of p-phenylenediamine, approximately 2.5 mole percent of m-phenylenediamine, approximately 35 mole percent of 3,3',4,4'-benzophenonetetracarboxylic dianhydride, and approximately 15 mole percent of the 3,3'-diethylester of 3,3',4,4'-benzophenonetetracarboxylic acid wherein said polyamic acid oligomer is an intermediate in the formation of said rigid polyimide.

13. A carbon fiber having a flexible coating on the surface thereof in a concentration of approximately 0.5 to 1.3 percent by weight based upon the weight of the carbon fiber.

14. A composite structure comprising a rigid polyimide matrix having carbon fibers incorporated therein which are coated on the surface thereof with approximately 0.3 to 5.0 percent by weight based upon the

5 weight of the carbon fibers of a sizing composition comprising a rigid polyimide coating which is derived from the reaction of at least one aromatic diamine, at least one aromatic dianhydride, and at least one aromatic tetracarboxylic acid diester in which the carboxylic acid groups and ester groups are ortho disposed, wherein a polyamic acid oligomer is formed as an intermediate during the formation of said rigid polyimide coating and is present within a flexible coating comprising said reactants which facilitates impregnation of said coated carbon fibers with said matrix during the formation of said composite structure.

10 15 16 17 18 19 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 1

from the reaction of approximately 47.5 mole percent of p-phenylenediamine, approximately 2.5 mole percent of m-phenylenediamine, approximately 35 mole percent of 3,3',4,4'-benzophenonetetracarboxylic dianhydride, and approximately 15 mole percent of the 3,3'-diethylester of 3,3',4,4'-benzophenonetetracarboxylic acid, wherein a polyamic acid oligomer is formed as an intermediate during the formation of said rigid polyimide coating and is present within a flexible coating comprising said reac-

tants which facilitates impregnation of said coated carbon fibers with said matrix during the formation of said composite structure.

26. A composite structure according to claim 25 wherein said carbon fibers are coated on the surface thereof with approximately 0.5 to 1.3 percent weight based upon the weight of the carbon fibers of said sizing composition comprising a rigid polyimide.

\* \* \* \* \*

10

15

20

25

30

35

40

45

50

55

60

65